

C. TURNER.

PROCESS OF DESTRUCTIVE DISTILLATION.

APPLICATION FILED JUNE 12, 1918.

1,336,264.

Patented Apr. 6, 1920.



Witnesses

C. A. Steele

Morris L. Gumbley.

Inventor  
Charles Turner  
by  
John L. Penry  
Attorney

# UNITED STATES PATENT OFFICE.

CHARLES TURNER, OF IRLAM, ENGLAND.

## PROCESS OF DESTRUCTIVE DISTILLATION.

1,336,264.

Specification of Letters Patent.

Patented Apr. 6, 1920.

Application filed June 12, 1918. Serial No. 239,637.

To all whom it may concern:

Be it known that I, CHARLES TURNER, a subject of the King of Great Britain, residing in Irlam, England, have invented certain new and useful Improvements in Processes of Destructive Distillation, of which the following is a specification.

I have discovered that destructive distillation of carbonaceous materials, such as wood, peat, lignite, oil shale, or coal, may be advantageously conducted in a vessel which is alternately closed until the pressure therein has attained a desired maximum and then opened, whereby the pressure is reduced rapidly from this maximum. By the term "destructive distillation" I do not include the cracking of hydrocarbon oils by heating the liquid oil in mass.

The products obtained by conducting the destructive distillation in this manner may be different in respect of proportion or nature or both from those obtained when the pressure is not purposely varied, the outstanding difference in the case of most kinds of carbonaceous materials being the larger proportion of oils and smaller proportion of pitch.

The invention is applicable with any mode of heating, whether external or internal, but inasmuch as the known method of heating which consists in passing heated elastic fluid over or through the material in the vessel, affords particular facility for varying the pressure within the vessel, this mode of heating is generally preferable.

The invention may be applied for instance by charging the material into a retort or like container having one or more inlets for a heating agent, such as superheated steam, and one or more outlets for the agent and the volatile products of carbonization which accompany it. The outlet is alternately closed or throttled and opened for passage of the elastic fluids by, for instance, a suitable valve which may be automatically operated by known mechanism depending for its action on the pressure within the container or on some external force. The superheated steam or other heated elastic fluid is passed into the container for a certain period of time or until the pressure as indicated by a manometer has risen to the required value. The valve then opens or is opened for a certain period of time or long enough to allow the pressure within the container to fall to that which has been decided upon as the lower limit.

The outlet from the container is connected with any suitable system of plant for collecting products of carbonization constructed in respect of dimensions with due regard to 60 the sudden flow of products and agents at each reduction of pressure.

Since the alternation of pressure is the cause of the beneficial effect of the invention, it is in most cases possible to vary considerably the absolute initial and final pressures chosen, and when it is known to be advantageous to carbonize under pressures below that of the atmosphere the invention is still applicable provided such pressures 70 are alternately lowered and raised.

The invention is applicable to processes of continuous and semi-continuous carbonization as well as to processes of intermittent carbonization. Obviously in continuous processes greater attention than usual must be paid to the gas-tight character of the charging and discharging devices.

The invention being applicable to a variety of carbonaceous materials, requiring, 80 as is known, different conditions of temperature and rate of carbonization, both of which affect the range of pressure and the periods of alternation according to this invention, it is impossible here to prescribe 85 the best conditions for operating; these can be determined only by experiment with due regard to the nature and proportion of products required.

As a specific example, however, I will recite the procedure I have adopted in carbonizing peat with the object of obtaining the maximum yield of oils, the accompanying drawing being a diagrammatic axial section through the retort used.

A cylindrical iron retort *a* 2½ feet in diameter and 7 feet high is connected at *b* through a stop valve with a boiler (not shown) adapted to generate steam at 20 lbs. pressure above atmospheric, and at *c* 95 through a stop valve *d* with a condensing plant (not shown). This retort is provided with a manometer *e* and is preferably jacketed with a bad conductor of heat. It is charged through a rotary feeding device *f* 100 with air-dried peat which has been coarsely disintegrated and supplied to hopper *g*; it is discharged by a revolving screw *h* which extracts the carbonized peat and delivers it into the delivery chute *i*. Both the feeding 105 device and the discharging screw are adapted to prevent leakage from the retort.

- during the heating operation. When the retort has been charged steam is blown in at *b* while valve *d* is open, until the air in the retort has been expelled. Valve *d* is now closed and steam from the boiler is passed through a superheater capable of raising its temperature to 500° C. and into the container until the manometer indicates 5 lbs. per square inch pressure; the valve *b* is now closed and valve *d* opened, by hand, until the pressure as indicated by the manometer has fallen to 2 lbs. per square inch, whereupon the valve *d* is closed and the inlet valve opened and the pressure allowed to rise again to 5 lbs. per square inch, and so on, the operations being repeated until observation of the condensing plant shows that there is no longer any substantial distillation of products.
- Having thus described the nature of the said invention and the best means I know of carrying the same into practical effect, I claim:
1. A process of destructive distillation of solid carbonaceous material, which process consists in heating a charge of the material in a closed vessel until the elastic fluid pressure therein has attained a selected maximum and thereupon relieving the pressure in the vessel by causing the elastic fluid to expand

into a condenser, and repeating these operations upon the same charge until distillation is complete.

2. A process of destructive distillation of solid carbonaceous material, which process consists in passing into a vessel containing a charge of the material a heated elastic fluid until the elastic fluid pressure within the vessel has attained a selected maximum and thereupon relieving the pressure within the vessel by causing the elastic fluid to expand into a condenser, and repeating these operations upon the same charge until distillation is complete.

3. A process of destructive distillation of solid carbonaceous material, which process consists in passing into a closed vessel containing a charge of the material superheated steam so that the elastic fluid pressure within the vessel rises to a selected maximum and thereupon opening the vessel to a condenser and repeating these operations until distillation is complete.

In testimony whereof I have signed my name to this specification in the presence of two subscribing witnesses.

CHARLES TURNER.

Witnesses:

JAMES LEITCH,  
JOHN EDDIE SMITH.